



US011126099B2

(12) **United States Patent**  
**Yamagishi et al.**

(10) **Patent No.:** US 11,126,099 B2  
(45) **Date of Patent:** Sep. 21, 2021

(54) **ELECTROSTATIC-IMAGE DEVELOPING TONER, ELECTROSTATIC-IMAGE DEVELOPER, TONER CARTRIDGE, PROCESS CARTRIDGE, IMAGE FORMING APPARATUS, AND IMAGE FORMING METHOD**

(71) **Applicant:** FUJIFILM Business Innovation Corp., Tokyo (JP)

(72) **Inventors:** Yuka Yamagishi, Kanagawa (JP); Daisuke Noguchi, Kanagawa (JP); Sakiko Takeuchi, Kanagawa (JP); Kazuhiko Nakamura, Kanagawa (JP); Yutaka Saito, Kanagawa (JP)

(73) **Assignee:** FUJIFILM Business Innovation Corp., Tokyo (JP)

(\*) **Notice:** Subject to any disclaimer, the term of this patent is extended or adjusted under 35 U.S.C. 154(b) by 0 days.

(21) **Appl. No.:** 16/842,734

(22) **Filed:** Apr. 7, 2020

(65) **Prior Publication Data**

US 2021/0088921 A1 Mar. 25, 2021

(30) **Foreign Application Priority Data**

Sep. 19, 2019 (JP) ..... JP2019-170504

(51) **Int. Cl.**

G03G 9/08 (2006.01)  
G03G 21/00 (2006.01)  
G03G 15/08 (2006.01)  
G03G 15/20 (2006.01)  
G03G 15/02 (2006.01)

G03G 9/113 (2006.01)  
G03G 9/097 (2006.01)  
(52) **U.S. Cl.**  
CPC ..... G03G 9/0827 (2013.01); G03G 9/0819 (2013.01); G03G 9/0821 (2013.01); G03G 9/09708 (2013.01); G03G 9/1138 (2013.01); G03G 9/1139 (2013.01); G03G 15/02 (2013.01); G03G 15/0865 (2013.01); G03G 15/20 (2013.01); G03G 21/0011 (2013.01)

(58) **Field of Classification Search**  
CPC ..... G03G 9/09708; G03G 9/1138; G03G 9/1139; G03G 9/0819; G03G 9/0821  
USPC ..... 430/108.1  
See application file for complete search history.

(56) **References Cited**

U.S. PATENT DOCUMENTS

2017/0227860 A1 \* 8/2017 Eri ..... G03G 15/08

FOREIGN PATENT DOCUMENTS

JP 2006317489 11/2006  
JP 2009-237274 10/2009

\* cited by examiner

*Primary Examiner* — Mark A Chapman

(74) *Attorney, Agent, or Firm* — JCIPRNET

(57) **ABSTRACT**

An electrostatic-image developing toner includes toner particles, layered compound particles, and inorganic particles. The inorganic particles have an average circularity of 0.910 or more and 0.995 or less. A ratio Da/Db of a number-average particle size Da of the layered compound particles to a number-average particle size Db of the inorganic particles is 1.2 or more and 43 or less.

20 Claims, 2 Drawing Sheets



FIG. 1



FIG. 2



## 1

**ELECTROSTATIC-IMAGE DEVELOPING  
TONER, ELECTROSTATIC-IMAGE  
DEVELOPER, TONER CARTRIDGE,  
PROCESS CARTRIDGE, IMAGE FORMING  
APPARATUS, AND IMAGE FORMING  
METHOD**

**CROSS-REFERENCE TO RELATED  
APPLICATIONS**

This application is based on and claims priority under 35 USC 119 from Japanese Patent Application No. 2019-170504 filed Sep. 19, 2019.

**BACKGROUND**

(i) Technical Field

The present disclosure relates to an electrostatic-image developing toner, an electrostatic-image developer, a toner cartridge, a process cartridge, an image forming apparatus, and an image forming method.

(ii) Related Art

Japanese Laid Open Patent Application Publication No. 2006-317489 discloses a toner that includes toner base particles having an average circularity of 0.94 to 0.995 and a volume-average particle size of 3 to 9  $\mu\text{m}$  and melamine cyanurate powder particles having a volume-average particle size of 3 to 9  $\mu\text{m}$  which are deposited on the toner base particles such that the amount of the melamine cyanurate powder particles is 0.1 to 2.0 parts by weight relative to 100 parts by weight of the toner base particles.

Japanese Laid Open Patent Application Publication No. 2009-237274 discloses a positively chargeable toner that includes colored resin particles including a binder resin, a colorant, and a positively-charging control agent and melamine cyanurate particles having a number-average primary particle size of 0.05 to 1.5  $\mu\text{m}$  which are deposited on the colored resin particles such that the amount of the melamine cyanurate particles is 0.01 to 0.5 parts by weight relative to 100 parts by weight of the colored resin particles.

**SUMMARY**

Aspects of non-limiting embodiments of the present disclosure relate to an electrostatic-image developing toner that may reduce the formation of colored streaks, which is caused by aggregates of layered compound particles, compared with an electrostatic-image developing toner that includes toner particles, layered compound particles, and inorganic particles, wherein the inorganic particles have an average circularity of less than 0.910, or wherein the ratio Da/Db of the number-average particle size Da of the layered compound particles to the number-average particle size Db of the inorganic particles is less than 1.2 or more than 43.

Aspects of certain non-limiting embodiments of the present disclosure address the above advantages and/or other advantages not described above. However, aspects of the non-limiting embodiments are not required to address the advantages described above, and aspects of the non-limiting embodiments of the present disclosure may not address advantages described above.

According to an aspect of the present disclosure, there is provided an electrostatic-image developing toner including toner particles, layered compound particles, and inorganic

## 2

particles. The inorganic particles have an average circularity of 0.910 or more and 0.995 or less. A ratio Da/Db of a number-average particle size Da of the layered compound particles to a number-average particle size Db of the inorganic particles is 1.2 or more and 43 or less.

**BRIEF DESCRIPTION OF THE DRAWINGS**

An exemplary embodiment of the present disclosure will 10 be described in detail based on the following figures, wherein:

FIG. 1 is a schematic diagram illustrating an example of an image forming apparatus according to an exemplary embodiment; and

15 FIG. 2 is a schematic diagram illustrating an example of a process cartridge according to an exemplary embodiment which is detachably attachable to an image forming apparatus.

**DETAILED DESCRIPTION**

An exemplary embodiment of the present disclosure is described below. The following description and Examples 20 below are intended to be illustrative of the exemplary embodiment and not restrictive of the scope of the exemplary embodiment.

In the present disclosure, a numerical range expressed using “to” means the range specified by the minimum and maximum described before and after “to”, respectively.

30 In the present disclosure, when numerical ranges are described in a stepwise manner, the upper or lower limit of a numerical range may be replaced with the upper or lower limit of another numerical range, respectively. In the present disclosure, the upper and lower limits of a numerical range 35 may be replaced with the upper and lower limits described in Examples below.

The term “step” used herein refers not only to an individual step but also to a step that is not distinguishable from other steps but achieves the intended purpose of the step.

40 In the present disclosure, when an exemplary embodiment is described with reference to a drawing, the structure of the exemplary embodiment is not limited to the structure illustrated in the drawing. The sizes of the members illustrated in the attached drawings are conceptual and do not limit the 45 relative relationship among the sizes of the members.

Each of the components described in the present disclosure may include plural types of substances that correspond to the component. In the present disclosure, in the case where a composition includes plural substances that correspond to a component of the composition, the content of the component in the composition is the total content of the 50 plural substances in the composition unless otherwise specified.

In the present disclosure, the number of types of particles 55 that correspond to a component may be two or more. In the case where a composition includes plural types of particles that correspond to a component of the composition, the particle size of the component is the particle size of a mixture of the plural types of particles included in the 60 composition unless otherwise specified.

In the present disclosure, an electrostatic-image developing toner may be referred to simply as “toner”, and an electrostatic-image developer may be referred to simply as “developer”.

65 **Electrostatic-Image Developing Toner**

A toner according to the exemplary embodiment includes toner particles, layered compound particles, and inorganic

particles. The inorganic particles have an average circularity of 0.910 or more and 0.995 or less. The ratio Da/Db of the number-average particle size Da of the layered compound particles to the number-average particle size Db of the inorganic particles is 1.2 or more and 43 or less.

The toner according to the exemplary embodiment may reduce the formation of colored streaks which is caused by aggregates of layered compound particles. The mechanisms for this are presumably as described below.

Toners that include layered compound particles, such as melamine cyanurate particles and boron nitride particles, used as an external additive are known. The layered compound particles are particles of a compound having a layered structure with an interlayer distance of the order of angstroms and are considered to produce a lubricating effect as a result of the layers becoming displaced with respect to one another. The layered compound particles deposited on the toner particles as an external additive serve as a lubricant at the point at which an image holding member and a cleaning blade come into contact with each other.

However, under the condition where a cleaning blade is excessively drawn in the direction in which an image holding member rotates, such as when a high-density image is continuously formed for a long period of time in a high-temperature, high-humidity environment (e.g., at 28°C. and a relative humidity of 85%), a large force is applied to the edge of the cleaning blade, which compresses the gaps between the layers of the layered compound particles and causes the layered compound particles to compress one another. As a result, aggregates are formed. The aggregates of the layered compound particles may slip through the cleaning blade and cause colored streaks to be formed in an image.

In order to address the above issue, in the exemplary embodiment, the size of the inorganic particles deposited on the toner particles as an external additive in addition to the layered compound particles is limited to fall within the adequate range, that is, the ratio Da/Db of the number-average particle size Da of the layered compound particles to the number-average particle size Db of the inorganic particles is 1.2 or more and 43 or less. This may enable the inorganic particles to enter the gaps between the layered compound particles and thereby reduce the aggregation of the layered compound particles.

Furthermore, the average circularity of the inorganic particles is 0.910 or more, that is, the inorganic particles are spherical inorganic particles having a high circularity. This enables the inorganic particles interposed between the layered compound particles to serve as rollers and enhance the lubricity of the layered compound particles. Consequently, a reduction in the lubricating effect of the layered compound particles may be limited even when a high-density image is continuously formed for a long period of time in a high-temperature, high-humidity environment. Moreover, since the inorganic particles serve as rollers, the aggregation of the layered compound particles may be reduced.

Accordingly, the toner according to the exemplary embodiment may reduce the aggregation of the layered compound particles at the point at which an image holding member and a cleaning blade come into contact with each other, enable the lubricating effect of the layered compound particles to be maintained, and reduce the formation of the colored streaks.

In the toner according to the exemplary embodiment, the ratio Da/Db of the number-average particle size Da of the layered compound particles to the number-average particle

size Db of the inorganic particles is 1.2 or more and 43 or less in order to reduce the aggregation of the layered compound particles.

If the ratio Da/Db is less than 1.2, the likelihood of the inorganic particles entering the gaps between the layered compound particles may be reduced since the inorganic particles are excessively large compared with the layered compound particles.

If the ratio Da/Db is more than 43, the inorganic particles may become buried in the surfaces of the layered compound particles and fail to serve as rollers since the inorganic particles are excessively small compared with the layered compound particles.

For the above reasons, the ratio Da/Db is 1.2 or more and 43 or less, is more preferably 5 or more and 43 or less, and is further preferably 10 or more and 43 or less.

In the toner according to the exemplary embodiment, the average circularity of the inorganic particles deposited on the toner particles as an external additive in addition to the layered compound particles is 0.910 or more in order to enable the inorganic particles to serve as rollers in the gaps between the layered compound particles. If the average circularity of the inorganic particles is less than 0.910, that is, if the inorganic particles are deformed inorganic particles having a low circularity, the performance of the inorganic particles as rollers may become degraded. The average circularity of the inorganic particles is preferably 0.920 or more, is more preferably 0.930 or more, and is further preferably 0.940 or more.

Although the average circularity of the inorganic particles is desirably increased to the maximum in order to use the inorganic particles as rollers, it is not easy to make all the inorganic particles perfectly spherical (i.e., an average circularity of 1). The average circularity of the inorganic particles is practically 0.995 or less.

The mass ratio Mb/Ma of the content Mb of the inorganic particles to the content Ma of the layered compound particles is preferably 0.1 or more and 500 or less, is more preferably 1 or more and 500 or less, and is further preferably 5 or more and 500 or less in order to enable the above-described mechanisms to work in an efficient manner and reduce the aggregation of the layered compound particles.

Details of the components, structure, and properties of the toner according to the exemplary embodiment are described below.

#### Toner Particles

The toner particles include, for example, a binder resin and may optionally include a colorant, a release agent, and other additives.

#### Binder Resin

Examples of the binder resin include vinyl resins that are homopolymers of the following monomers or copolymers of two or more monomers selected from the following monomers: styrenes, such as styrene, para-chlorostyrene, and  $\alpha$ -methylstyrene; (meth)acrylates, such as methyl acrylate, ethyl acrylate, n-propyl acrylate, n-butyl acrylate, lauryl acrylate, 2-ethylhexyl acrylate, methyl methacrylate, ethyl methacrylate, n-propyl methacrylate, lauryl methacrylate, and 2-ethylhexyl methacrylate; ethylenically unsaturated nitriles, such as acrylonitrile and methacrylonitrile; vinyl ethers, such as vinyl methyl ether and vinyl isobutyl ether; vinyl ketones, such as vinyl methyl ketone, vinyl ethyl ketone, and vinyl isopropenyl ketone; and olefins, such as ethylene, propylene, and butadiene.

Examples of the binder resin further include non-vinyl resins, such as epoxy resins, polyester resins, polyurethane

resins, polyamide resins, cellulose resins, polyether resins, and modified rosins; a mixture of the non-vinyl resin and the vinyl resin; and a graft polymer produced by polymerization of the vinyl monomer in the presence of the non-vinyl resin.

The above binder resins may be used alone or in combination of two or more.

The binder resin may be a polyester resin.

Examples of the polyester resin include amorphous polyester resins known in the related art. A crystalline polyester resin may be used as a polyester resin in combination with an amorphous polyester resin. In such a case, the content of the crystalline polyester resin in the binder resin may be 2% by mass or more and 40% by mass or less and is preferably 2% by mass or more and 20% by mass or less.

The term "crystalline" resin used herein refers to a resin that, in thermal analysis using differential scanning calorimetry (DSC), exhibits a distinct endothermic peak instead of step-like endothermic change and specifically refers to a resin that exhibits an endothermic peak with a half-width of 10° C. or less at a heating rate of 10° C./min.

On the other hand, the term "amorphous" resin used herein refers to a resin that exhibits an endothermic peak with a half-width of more than 10° C., that exhibits step-like endothermic change, or that does not exhibit a distinct endothermic peak.

#### Amorphous Polyester Resin

Examples of the amorphous polyester resin include condensation polymers of a polyvalent carboxylic acid and a polyhydric alcohol. The amorphous polyester resin may be a commercially available one or a synthesized one.

Examples of the polyvalent carboxylic acid include aliphatic dicarboxylic acids, such as oxalic acid, malonic acid, maleic acid, fumaric acid, citraconic acid, itaconic acid, glutaconic acid, succinic acid, alkenyl succinic acid, adipic acid, and sebamic acid; alicyclic dicarboxylic acids, such as cyclohexanedicarboxylic acid; aromatic dicarboxylic acids, such as terephthalic acid, isophthalic acid, phthalic acid, and naphthalenedicarboxylic acid; anhydrides of these dicarboxylic acids; and lower (e.g., 1 to 5 carbon atoms) alkyl esters of these dicarboxylic acids. Among these dicarboxylic acids, for example, aromatic dicarboxylic acids may be used as a polyvalent carboxylic acid.

Trivalent or higher carboxylic acids having a crosslinked structure or a branched structure may be used as a polyvalent carboxylic acid in combination with the dicarboxylic acids. Examples of the trivalent or higher carboxylic acids include trimellitic acid, pyromellitic acid, anhydrides of these carboxylic acids, and lower (e.g., 1 to 5 carbon atoms) alkyl esters of these carboxylic acids.

The above polyvalent carboxylic acids may be used alone or in combination of two or more.

Examples of the polyhydric alcohol include aliphatic diols, such as ethylene glycol, diethylene glycol, triethylene glycol, propylene glycol, butanediol, hexanediol, and neopentyl glycol; alicyclic diols, such as cyclohexanediol, cyclohexanedimethanol, and hydrogenated bisphenol A; and aromatic diols, such as bisphenol A-ethylene oxide adduct and bisphenol A-propylene oxide adduct. Among these diols, for example, aromatic diols and alicyclic diols may be used as a polyhydric alcohol. In particular, aromatic diols may be used as a polyhydric alcohol.

Trihydric or higher alcohols having a crosslinked structure or a branched structure may be used as a polyhydric alcohol in combination with the diols. Examples of the trihydric or higher alcohols include glycerin, trimethylolpropane, and pentaerythritol.

The above polyhydric alcohols may be used alone or in combination of two or more.

The glass transition temperature Tg of the amorphous polyester resin is preferably 50° C. or more and 80° C. or less and is more preferably 50° C. or more and 65° C. or less.

The glass transition temperature is determined from a DSC curve obtained by differential scanning calorimetry (DSC). More specifically, the glass transition temperature is determined from the "extrapolated glass-transition-starting temperature" according to a method for determining glass transition temperature which is described in JIS K 7121: 1987 "Testing Methods for Transition Temperatures of Plastics".

The weight-average molecular weight Mw of the amorphous polyester resin is preferably 5,000 or more and 1,000,000 or less and is more preferably 7,000 or more and 500,000 or less.

The number-average molecular weight Mn of the amorphous polyester resin is preferably 2,000 or more and 100,000 or less.

The molecular weight distribution index Mw/Mn of the amorphous polyester resin is preferably 1.5 or more and 100 or less and is more preferably 2 or more and 60 or less.

The weight-average molecular weight and number-average molecular weight of the amorphous polyester resin are determined by gel permeation chromatography (GPC). Specifically, the molecular weights of the amorphous polyester resin are determined by GPC using a "HLC-8120GPC" produced by Tosoh Corporation as measuring equipment, a column "TSKgel SuperHM-M (15 cm)" produced by Tosoh Corporation, and a tetrahydrofuran (THF) solvent. The weight-average molecular weight and number-average molecular weight of the amorphous polyester resin are determined on the basis of the results of the measurement using a molecular-weight calibration curve based on monodisperse polystyrene standard samples.

The amorphous polyester resin may be produced by any suitable production method known in the related art. Specifically, the amorphous polyester resin may be produced by, for example, a method in which polymerization is performed at 180° C. or more and 230° C. or less, the pressure inside the reaction system is reduced as needed, and water and alcohols that are generated by condensation are removed.

In the case where the raw materials, that is, the monomers, are not dissolved in or miscible with each other at the reaction temperature, a solvent having a high boiling point may be used as a dissolution adjuvant in order to dissolve the raw materials. In such a case, the condensation polymerization reaction is performed while the dissolution adjuvant is distilled away. In the case where the monomers used in the copolymerization reaction have low miscibility with each other, a condensation reaction of the monomers with an acid or alcohol that is to undergo a polycondensation reaction with the monomers may be performed in advance and subsequently polycondensation of the resulting polymers with the other components may be performed.

#### Crystalline Polyester Resin

Examples of the crystalline polyester resin include condensation polymers of a polyvalent carboxylic acid and a polyhydric alcohol. The crystalline polyester resin may be commercially available one or a synthesized one.

In order to increase ease of forming a crystal structure, a condensation polymer prepared from linear aliphatic polymerizable monomers may be used as a crystalline polyester resin instead of a condensation polymer prepared from polymerizable monomers having an aromatic ring.

Examples of the polyvalent carboxylic acid include aliphatic dicarboxylic acids, such as oxalic acid, succinic acid, glutaric acid, adipic acid, suberic acid, azelaic acid, sebacic acid, 1,9-nonanedicarboxylic acid, 1,10-decanedicarboxylic acid, 1,12-dodecanedicarboxylic acid, 1,14-tetradecanedicarboxylic acid, and 1,18-octadecanedicarboxylic acid; aromatic dicarboxylic acids, such as dibasic acids (e.g., phthalic acid, isophthalic acid, terephthalic acid, and naphthalene-2, 6-dicarboxylic acid); anhydrides of these dicarboxylic acids; and lower (e.g., 1 to 5 carbon atoms) alkyl esters of these dicarboxylic acids.

Trivalent or higher carboxylic acids having a crosslinked structure or a branched structure may be used as a polyvalent carboxylic acid in combination with the dicarboxylic acids. Examples of the trivalent carboxylic acids include aromatic carboxylic acids, such as 1,2,3-benzenetricarboxylic acid, 1,2,4-benzenetricarboxylic acid, and 1,2,4-naphthalenetricarboxylic acid; anhydrides of these tricarboxylic acids; and lower (e.g., 1 to 5 carbon atoms) alkyl esters of these tricarboxylic acids.

Dicarboxylic acids including a sulfonic group and dicarboxylic acids including an ethylenic double bond may be used as a polyvalent carboxylic acid in combination with the above dicarboxylic acids.

The above polyvalent carboxylic acids may be used alone or in combination of two or more.

Examples of the polyhydric alcohol include aliphatic diols, such as linear aliphatic diols including a backbone having 7 to 20 carbon atoms. Examples of the aliphatic diols include ethylene glycol, 1,3-propanediol, 1,4-butanediol, 1,5-pentanediol, 1,6-hexanediol, 1,7-heptanediol, 1,8-octanediol, 1,9-nonanediol, 1,10-decanediol, 1,11-undecanediol, 1,12-dodecanediol, 1,13-tridecanediol, 1,14-tetradecanediol, 1,18-octadecanediol, and 1,14-eicosanedecanediol. Among these aliphatic diols, 1,8-octanediol, 1,9-nonanediol, and 1,10-decanediol may be used.

Trihydric or higher alcohols having a crosslinked structure or a branched structure may be used as a polyhydric alcohol in combination with the above diols. Examples of the trihydric or higher alcohols include glycerin, trimethylolethane, trimethylolpropane, and pentaerythritol.

The above polyhydric alcohols may be used alone or in combination of two or more.

The content of the aliphatic diols in the polyhydric alcohol may be 80 mol % or more and is preferably 90 mol % or more.

The melting temperature of the crystalline polyester resin is preferably 50° C. or more and 100° C. or less, is more preferably 55° C. or more and 90° C. or less, and is further preferably 60° C. or more and 85° C. or less.

The melting temperature of the crystalline polyester resin is determined from the "melting peak temperature" according to a method for determining melting temperature which is described in JIS K 7121:1987 "Testing Methods for Transition Temperatures of Plastics" using a DSC curve obtained by differential scanning calorimetry (DSC).

The crystalline polyester resin may have a weight-average molecular weight Mw of 6,000 or more and 35,000 or less.

The crystalline polyester resin may be produced by any suitable method known in the related art similarly to, for example, the amorphous polyester resin.

The content of the binder resin in the toner particles is preferably 40% by mass or more and 95% by mass or less, is more preferably 50% by mass or more and 90% by mass or less, and is further preferably 60% by mass or more and 85% by mass or less.

#### Colorant

Examples of the colorant include pigments, such as Carbon Black, Chrome Yellow, Hansa Yellow, Benzidine Yellow, Threne Yellow, Quinoline Yellow, Pigment Yellow, Permanent Orange GTR, Pyrazolone Orange, Vulcan Orange, Watching Red, Permanent Red, Brilliant Carmine 3B, Brilliant Carmine 6B, DuPont Oil Red, Pyrazolone Red, Lithol Red, Rhodamine B Lake, Lake Red C, Pigment Red, Rose Bengal, Aniline Blue, Ultramarine Blue, Calco Oil Blue, Methylene Blue Chloride, Phthalocyanine Blue, Pigment Blue, Phthalocyanine Green, and Malachite Green Oxalate; and dyes, such as acridine dyes, xanthene dyes, azo dyes, benzoquinone dyes, azine dyes, anthraquinone dyes, thioindigo dyes, dioxazine dyes, thiazine dyes, azomethine dyes, indigo dyes, phthalocyanine dyes, aniline black dyes, polymethine dyes, triphenylmethane dyes, diphenylmethane dyes, and thiazole dyes.

The above colorants may be used alone or in combination of two or more.

The colorant may optionally be subjected to a surface treatment and may be used in combination with a dispersant. Plural types of colorants may be used in combination.

The content of the colorant in the toner particles is preferably 1% by mass or more and 30% by mass or less and is more preferably 3% by mass or more and 15% by mass or less.

#### Release Agent

Examples of the release agent include, but are not limited to, hydrocarbon waxes; natural waxes, such as a carnauba wax, a rice bran wax, and a candelilla wax; synthetic or mineral-petroleum-derived waxes, such as a montan wax; and ester waxes, such as a fatty-acid ester wax and a montanate wax.

The melting temperature of the release agent is preferably 50° C. or more and 110° C. or less and is more preferably 60° C. or more and 100° C. or less.

The melting temperature of the release agent is determined from the "melting peak temperature" according to a method for determining melting temperature which is described in JIS K 7121:1987 "Testing Methods for Transition Temperatures of Plastics" using a DSC curve obtained by differential scanning calorimetry (DSC).

The content of the release agent in the toner particles is preferably 1% by mass or more and 20% by mass or less and is more preferably 5% by mass or more and 15% by mass or less.

#### Other Additives

Examples of the other additives include additives known in the related art, such as a magnetic substance, a charge-controlling agent, and an inorganic powder. These additives may be added to the toner particles as internal additives.

#### Properties, etc. of Toner Particles

The toner particles may have a single-layer structure or a "core-shell" structure constituted by a core (i.e., core particle) and a coating layer (i.e., shell layer) covering the core.

The core-shell structure of the toner particles may be constituted by, for example, a core including a binder resin and, as needed, other additives such as a colorant and a release agent and by a coating layer including the binder resin.

The volume-average diameter D50v of the toner particles is preferably 2 µm or more and 10 µm or less and is more preferably 4 µm or more and 8 µm or less.

The above-described average diameters and particle diameter distribution indices of the toner particles are measured using "COULTER Multisizer II" (produced by Beck-

man Coulter, Inc.) with an electrolyte "ISOTON-II" (produced by Beckman Coulter, Inc.) in the following manner.

A sample to be measured (0.5 mg or more and 50 mg or less) is added to 2 ml of a 5 mass %-aqueous solution of a surfactant (e.g., sodium alkylbenzene sulfonate) that serves as a dispersant. The resulting mixture is added to 100 ml or more and 150 ml or less of an electrolyte.

The resulting electrolyte containing the sample suspended therein is subjected to a dispersion treatment for 1 minute using an ultrasonic disperser, and the distribution of the diameters of particles having a diameter of 2  $\mu\text{m}$  or more and 60  $\mu\text{m}$  or less is measured using COULTER Multisizer II with an aperture having a diameter of 100  $\mu\text{m}$ . The number of the particles sampled is 50,000.

The particle diameter distribution measured is divided into a number of particle diameter ranges (i.e., channels). For each range, in ascending order in terms of particle diameter, the cumulative volume and the cumulative number are calculated and plotted to draw cumulative distribution curves. Particle diameters at which the cumulative volume and the cumulative number reach 16% are considered to be the volume particle diameter D16v and the number particle diameter D16p, respectively. Particle diameters at which the cumulative volume and the cumulative number reach 50% are considered to be the volume-average particle diameter D50v and the number-average particle diameter D50p, respectively. Particle diameters at which the cumulative volume and the cumulative number reach 84% are considered to be the volume particle diameter D84v and the number particle diameter D84p, respectively.

Using the volume particle diameters and number particle diameters measured, the volume grain size distribution index (GSDv) is calculated as  $(\text{D84v}/\text{D16v})^{1/2}$  and the number grain size distribution index (GSDp) is calculated as  $(\text{D84p}/\text{D16p})^{1/2}$ .

The toner particles preferably has an average circularity of 0.94 or more and 1.00 or less. The average circularity of the toner particles is more preferably 0.95 or more and 0.98 or less.

The average circularity of the toner particles is determined as  $[\text{Equivalent circle perimeter}]/[\text{Perimeter}]$  (i.e.,  $[\text{Perimeter of a circle having the same projection area as the particles}]/[\text{Perimeter of the projection image of the particles}]$ ). Specifically, the average circularity of the toner particles is determined by the following method.

The toner particles to be measured are sampled by suction so as to form a flat stream. A static image of the particles is taken by instantaneously flashing a strobe light. The image of the particles is analyzed with a flow particle image analyzer "FPIA-3000" produced by Sysmex Corporation. The number of samples used for determining the average circularity of the toner particles is 3,500.

In the case where the toner includes an external additive, the toner (i.e., the developer) to be measured is dispersed in water containing a surfactant and then subjected to an ultrasonic wave treatment in order to remove the external additive from the toner particles.

#### Layered Compound Particles

The layered compound particles are particles of a compound having a layered structure. Examples of the layered compound particles include melamine cyanurate particles, boron nitride particles, graphite fluoride particles, molybdenum disulfide particles, and mica particles.

The number-average particle size Da of the layered compound particles is preferably 0.3  $\mu\text{m}$  or more and 5.0  $\mu\text{m}$  or less, is more preferably 0.3  $\mu\text{m}$  or more and 4.0  $\mu\text{m}$  or less, is further preferably 0.4  $\mu\text{m}$  or more and 3.0  $\mu\text{m}$  or less, and

is most preferably 0.4  $\mu\text{m}$  or more and 2.0  $\mu\text{m}$  or less in order to reduce the aggregation of the layered compound particles. The number-average particle size of the layered compound particles may be controlled by disintegration, classification, or a combination of disintegration and classification.

The number-average particle size Da of the layered compound particles is determined by the following measuring method.

First, the layered compound particles are separated from 10 the toner. The method for separating the layered compound particles from the toner is not limited. For example, an ultrasonic wave is applied to a dispersion liquid prepared by dispersing the toner particles in water containing a surfactant. The dispersion liquid is subjected to high-speed centrifugation to separate the toner particles, the layered compound particles, and the inorganic particles from one another by centrifugal force on the basis of specific gravity. The fraction containing the layered compound particles is extracted and dried to obtain layered compound particles.

15 The layered compound particles are added to an aqueous electrolyte solution (aqueous ISOTON solution). An ultrasonic wave is applied to the resulting mixture for 30 seconds or more in order to form a dispersion liquid. This dispersion liquid is used as a sample. The particle size of the layered compound particles is measured with a laser diffraction/scattering particle size distribution analyzer, such as "Microtrac MT3000II" produced by MicrotracBEL Corp. At least 3,000 layered compound particles are measured. The particle size at which the cumulative number reaches 50% in 20 a number grain size distribution drawn in ascending order in terms of particle size is considered the number-average particle size Da.

25 The content of the layered compound particles in the toner is preferably 0.01% by mass or more, is more preferably 0.02% by mass or more, is further preferably 0.05% by mass or more, and is most preferably 0.1% by mass or more of the total amount of the toner in order to produce the lubricating effect of the layered compound particles. The content of the layered compound particles in the toner is preferably 5.0% 30 by mass or less, is more preferably 1.0% by mass or less, is further preferably 0.7% by mass or less, and is most preferably 0.5% by mass or less of the total amount of the toner in order to reduce the aggregation of the layered compound particles.

#### 45 Inorganic Particles

40 Examples of the inorganic particles include  $\text{SiO}_2$  particles,  $\text{TiO}_2$  particles,  $\text{Al}_2\text{O}_3$  particles,  $\text{CuO}$  particles,  $\text{ZnO}$  particles,  $\text{SnO}_2$  particles,  $\text{CeO}_2$  particles,  $\text{Fe}_2\text{O}_3$  particles,  $\text{MgO}$  particles,  $\text{BaO}$  particles,  $\text{CaO}$  particles,  $\text{K}_2\text{O}$  particles,  $\text{Na}_2\text{O}$  particles,  $\text{ZrO}_2$  particles,  $\text{CaO} \cdot \text{SiO}_2$  particles,  $\text{K}_2\text{O} \cdot (\text{TiO}_2)_n$  particles,  $\text{Al}_2\text{O}_3 \cdot 2\text{SiO}_2$  particles,  $\text{CaCO}_3$  particles,  $\text{MgCO}_3$  particles,  $\text{BaSO}_4$  particles, and  $\text{MgSO}_4$  particles.

45 The inorganic particles are preferably silica particles and are more preferably sol gel silica particles, considering that silica particles and sol gel silica particles have high circularities. The sol-gel method for producing sol gel silica particles is publicly known. The sol-gel method includes, for example, adding ammonia water dropwise to a liquid mixture of a tetraalkoxysilane, water, and an alcohol to prepare a silica sol suspension, extracting a wet silica gel from the silica sol suspension by centrifugal separation, and drying the wet silica gel to prepare silica particles. Examples of the tetraalkoxysilane include tetramethoxysilane, tetraethoxysilane, tetrapropoxysilane, and tetrabutoxysilane.

50 The surfaces of the inorganic particles may be subjected to a hydrophobic treatment. The hydrophobic treatment is performed by, for example, immersing the inorganic par-

ticles in a hydrophobizing agent. Examples of the hydrophobizing agent include, but are not limited to, a silane coupling agent, a silicone oil, a titanate coupling agent, and aluminum coupling agent. These hydrophobizing agents may be used alone or in combination of two or more. The amount of the hydrophobizing agent is commonly, for example, 1 part by mass or more and 10 parts by mass or less relative to 100 parts by mass of the inorganic particles.

The average circularity of the inorganic particles is 0.910 or more, is preferably 0.920 or more, is more preferably 0.930 or more, and is further preferably 0.940 or more in order to reduce the aggregation of the layered compound particles. The average circularity of the inorganic particles is 0.995 or less in consideration of ease of adjustment of circularity.

The number-average particle size  $D_b$  of the inorganic particles is preferably 0.06  $\mu\text{m}$  or more and 0.3  $\mu\text{m}$  or less, is more preferably 0.06  $\mu\text{m}$  or more and 0.25  $\mu\text{m}$  or less, and is further preferably 0.07  $\mu\text{m}$  or more and 0.2  $\mu\text{m}$  or less in order to reduce the aggregation of the layered compound particles.

The average circularity and number-average particle size  $D_b$  of the inorganic particles are determined by the following measuring method.

First, the inorganic particles are separated from the toner. The method for separating the inorganic particles from the toner is not limited. For example, an ultrasonic wave is applied to a dispersion liquid prepared by dispersing the toner particles in water containing a surfactant. The dispersion liquid is subjected to high-speed centrifugation to separate the toner particles, the layered compound particles, and the inorganic particles from one another by centrifugal force on the basis of specific gravity. The fraction containing the inorganic particles is extracted and dried to obtain inorganic particles.

Images of the above inorganic particles are taken with a scanning electron microscope (SEM). The images are analyzed to calculate the circularity ( $=4\pi \times [\text{Area of particle image}]/[\text{Perimeter of particles image}]^2$ ) and equivalent circle diameter ( $\mu\text{m}$ ) of each of randomly selected 1,000 primary particles.

The average circularity is the circularity at which the cumulative number reaches 50% in a number circularity distribution drawn in ascending order in terms of circularity.

The number-average particle size  $D_b$  is the equivalent circle diameter at which the cumulative number reaches 50% in a number equivalent circle diameter distribution drawn in ascending order in terms of equivalent circle diameter.

The content of the inorganic particles in the toner is preferably 0.3% by mass or more and 5.0% by mass or less, is more preferably 0.5% by mass or more and 3.0% by mass or less, and is further preferably 0.5% by mass or more and 2.5% by mass or less of the total amount of the toner in order to reduce the aggregation of the layered compound particles. Other External Additive

The toner according to the exemplary embodiment may optionally include an external additive other than the layered compound particles or the inorganic particles. Examples of the other external additive include particles of a resin, such as polystyrene, polymethyl methacrylate, or a melamine resin; and particles of a cleaning lubricant, such as a metal salt of a higher fatty acid, such as zinc stearate, or a fluorine-based high-molecular-weight compound.

In the case where the toner according to the exemplary embodiment includes an external additive other than the layered compound particles or the inorganic particles, the

total amount of the other external additives used is preferably 0.01% by mass or more and 5.0% by mass or less and is more preferably 0.01% by mass or more and 2.0% by mass or less of the amount of the toner particles.

5 Method for Producing Toner

The toner according to the exemplary embodiment is produced by, after the preparation of the toner particles, depositing an external additive on the surfaces of the toner particles.

10 The toner particles may be prepared by any dry process, such as knead pulverization, or any wet process, such as aggregation coalescence, suspension polymerization, or dissolution suspension. However, a method for preparing the toner particles is not limited thereto, and any suitable method known in the related art may be used. Among these methods, aggregation coalescence may be used in order to prepare the toner particles.

Specifically, in the case where, for example, aggregation 20 coalescence is used in order to prepare the toner particles, the toner particles are prepared by the following steps:

preparing a resin particle dispersion liquid in which resin 25 particles serving as a binder resin are dispersed (i.e., resin particle dispersion liquid preparation step);

causing the resin particles (and, as needed, other particles) 30 to aggregate together in the resin particle dispersion liquid (or in the resin particle dispersion liquid mixed with another particle dispersion liquid as needed) in order to form aggregated particles (i.e., aggregated particle formation step);

35 and heating the resulting aggregated particle dispersion liquid in which the aggregated particles are dispersed in order to cause fusion and coalescence of the aggregated particles to occur and thereby form toner particles (fusion-coalescence step).

35 Each of the above steps is described below in detail.

Hereinafter, a method for preparing toner particles including a colorant and a release agent is described. However, it should be noted that the colorant and the release agent are optional. It is needless to say that additives other than a colorant and a release agent may be used.

Resin Particle Dispersion Liquid Preparation Step

In addition to a resin particle dispersion liquid in which resin particles serving as a binder resin is dispersed, for example, a colorant particle dispersion liquid in which colorant particles are dispersed and a release-agent particle dispersion liquid in which release-agent particles are dispersed are prepared.

The resin particle dispersion liquid is prepared by, for example, dispersing resin particles in a dispersion medium using a surfactant.

Examples of the dispersion medium used for preparing the resin particle dispersion liquid include aqueous media.

Examples of the aqueous media include water, such as distilled water and ion-exchange water; and alcohols. These 55 aqueous media may be used alone or in combination of two or more.

Examples of the surfactant include anionic surfactants, such as sulfate-based surfactants, sulfonate-based surfactants, and phosphate-based surfactants; cationic surfactants, such as amine-salt-based surfactants and quaternary-ammonium-salt-based surfactants; and nonionic surfactants, such as polyethylene-glycol surfactants, alkylphenol-ethylene-oxide-adduct-based surfactants, and polyhydric-alcohol-based surfactants. Among these surfactants, in particular, the anionic surfactants and the cationic surfactants may be used. The nonionic surfactants may be used in combination with the anionic surfactants and the cationic surfactants.

## 13

These surfactants may be used alone or in combination of two or more.

In the preparation of the resin particle dispersion liquid, the resin particles can be dispersed in a dispersion medium by any suitable dispersion method commonly used in the related art in which, for example, a rotary-shearing homogenizer, a ball mill, a sand mill, or a dyno mill that includes media is used. Depending on the type of the resin particles used, the resin particles may be dispersed in the dispersion medium by, for example, phase-inversion emulsification. Phase-inversion emulsification is a method in which the resin to be dispersed is dissolved in a hydrophobic organic solvent in which the resin is soluble, a base is added to the resulting organic continuous phase (i.e., O phase) to perform neutralization, and subsequently an aqueous medium (i.e., W phase) is charged in order to perform phase inversion from W/O to O/W and disperse the resin in the aqueous medium in the form of particles.

The volume-average diameter of the resin particles dispersed in the resin particle dispersion liquid is preferably, for example, 0.01  $\mu\text{m}$  or more and 1  $\mu\text{m}$  or less, is more preferably 0.08  $\mu\text{m}$  or more and 0.8  $\mu\text{m}$  or less, and is further preferably 0.1  $\mu\text{m}$  or more and 0.6  $\mu\text{m}$  or less.

The volume-average diameter of the resin particles is determined in the following manner. The particle diameter distribution of the resin particles is obtained using a laser-diffraction particle-size-distribution measurement apparatus (e.g., "LA-700" produced by HORIBA, Ltd.). The particle diameter distribution measured is divided into a number of particle diameter ranges (i.e., channels). For each range, in ascending order in terms of particle diameter, the cumulative volume is calculated and plotted to draw a cumulative distribution curve. A particle diameter at which the cumulative volume reaches 50% is considered to be the volume particle diameter D50v. The volume-average diameters of particles included in the other dispersion liquids are also determined in the above-described manner.

The content of the resin particles included in the resin particle dispersion liquid is preferably 5% by mass or more and 50% by mass or less and is more preferably 10% by mass or more and 40% by mass or less.

The colorant particle dispersion liquid, the release-agent particle dispersion liquid, and the like are also prepared as in the preparation of the resin particle dispersion liquid. In other words, the above-described specifications for the volume-average diameter of the particles included in the resin particle dispersion liquid, the dispersion medium of the resin particle dispersion liquid, the dispersion method used for preparing the resin particle dispersion liquid, and the content of the particles in the resin particle dispersion liquid can also be applied to colorant particles dispersed in the colorant particle dispersion liquid and release-agent particles dispersed in the release-agent particle dispersion liquid.

#### Aggregated Particle Formation Step

The resin particle dispersion liquid is mixed with the colorant particle dispersion liquid and the release-agent particle dispersion liquid.

In the resulting mixed dispersion liquid, heteroaggregation of the resin particles with the colorant particles and the release-agent particles is performed in order to form aggregated particles including the resin particles, the colorant particles, and the release-agent particles, the aggregated particles having a diameter close to that of the desired toner particles.

Specifically, for example, a flocculant is added to the mixed dispersion liquid, and the pH of the mixed dispersion liquid is controlled to be acidic (e.g., pH of 2 or more and

## 14

5 or less). A dispersion stabilizer may be added to the mixed dispersion liquid as needed. Subsequently, the mixed dispersion liquid is heated to a temperature close to the glass transition temperature of the resin particles (specifically, e.g., [glass transition temperature of the resin particles—30° C.] or more and [the glass transition temperature—10° C.] or less), and thereby the particles dispersed in the mixed dispersion liquid are caused to aggregate together to form aggregated particles.

In the aggregated particle formation step, alternatively, for example, the above flocculant may be added to the mixed dispersion liquid at room temperature (e.g., 25° C.) while the mixed dispersion liquid is stirred using a rotary-shearing homogenizer. Then, the pH of the mixed dispersion liquid is controlled to be acidic (e.g., pH of 2 or more and 5 or less), and a dispersion stabilizer may be added to the mixed dispersion liquid as needed. Subsequently, the mixed dispersion liquid is heated in the above-described manner.

Examples of the flocculant include surfactants, inorganic metal salts, and divalent or higher metal complexes that have a polarity opposite to that of the surfactant included in the mixed dispersion liquid. Using a metal complex as a flocculant reduces the amount of surfactant used and, as a result, charging characteristics may be enhanced.

An additive capable of forming a complex or a bond similar to a complex with the metal ions contained in the flocculant may optionally be used in combination with the flocculant. An example of the additive is a chelating agent.

Examples of the inorganic metal salts include metal salts, such as calcium chloride, calcium nitrate, barium chloride, magnesium chloride, zinc chloride, aluminum chloride, and aluminum sulfate; and inorganic metal salt polymers, such as polyaluminum chloride, polyaluminum hydroxide, and calcium polysulfide.

The chelating agent may be a water-soluble chelating agent. Examples of such a chelating agent include oxycarboxylic acids, such as tartaric acid, citric acid, and gluconic acid; and aminocarboxylic acids, such as iminodiacetic acid (IDA), nitrilotriacetic acid (NTA), and ethylenediaminetetraacetic acid (EDTA).

The amount of the chelating agent used is preferably 0.01 parts by mass or more and 5.0 parts by mass or less and is more preferably 0.1 parts by mass or more and less than 3.0 parts by mass relative to 100 parts by mass of the resin particles.

#### Fusion-Coalescence Step

The aggregated particle dispersion liquid in which the aggregated particles are dispersed is heated to, for example, the glass transition temperature of the resin particles or more (e.g., temperature higher than the glass transition temperature of the resin particles by 10° C. to 30° C.) in order to perform fusion and coalescence of the aggregated particles. Hereby, toner particles are prepared.

The toner particles are prepared through the above-described steps.

It is also possible to prepare the toner particles by, after preparing the aggregated particle dispersion liquid in which the aggregated particles are dispersed, further mixing the aggregated particle dispersion liquid with a resin particle dispersion liquid in which resin particles are dispersed and subsequently performing aggregation such that the resin particles are deposited on the surfaces of the aggregated particles in order to form second aggregated particles; and by heating the resulting second-aggregated particle dispersion liquid in which the second aggregated particles are dispersed and thereby causing fusion and coalescence of the

## 15

second aggregated particles to occur in order to form toner particles having a core-shell structure.

After the completion of the fusion-coalescence step, the toner particles formed in the solution are subjected to any suitable cleaning step, solid-liquid separation step, and drying step that are known in the related art in order to obtain dried toner particles. In the cleaning step, the toner particles may be subjected to displacement washing using ion-exchange water to a sufficient degree from the viewpoint of electrification characteristics. Examples of a solid-liquid separation method used in the solid-liquid separation step include suction filtration and pressure filtration from the viewpoint of productivity. Examples of a drying method used in the drying step include freeze-drying, flash drying, fluidized drying, and vibrating fluidized drying from the viewpoint of productivity.

The toner according to the exemplary embodiment is produced by, for example, adding an external additive to the dried toner particles and mixing the resulting toner particles using a V-blender, a Henschel mixer, a Lodige mixer, or the like. Optionally, coarse toner particles may be removed using a vibrating screen classifier, a wind screen classifier, or the like.

## Electrostatic-Image Developer

The electrostatic-image developer according to the exemplary embodiment includes at least the toner according to the exemplary embodiment.

The electrostatic-image developer according to the exemplary embodiment may be a monocomponent developer including only the toner according to the exemplary embodiment or may be a two-component developer that is a mixture of the toner and a carrier.

The type of the carrier is not limited, and any suitable carrier known in the related art may be used. Examples of the carrier include a coated carrier prepared by coating the surfaces of cores including magnetic powder particles with a resin; a magnetic-powder-dispersed carrier prepared by dispersing and mixing magnetic powder particles in a matrix resin; and a resin-impregnated carrier prepared by impregnating a porous magnetic powder with a resin. The magnetic-powder-dispersed carrier and the resin-impregnated carrier may also be prepared by coating the surfaces of particles constituting the carrier, that is, core particles, with a resin.

Examples of the magnetic powder include powders of magnetic metals, such as iron, nickel, and cobalt; and powders of magnetic oxides, such as ferrite and magnetite.

Examples of the coat resin and the matrix resin include polyethylene, polypropylene, polystyrene, poly(vinyl acetate), poly(vinyl alcohol), poly(vinyl butyral), poly(vinyl chloride), poly(vinyl ether), poly(vinyl ketone), a vinyl chloride-vinyl acetate copolymer, a styrene-acrylic acid ester copolymer, a straight silicone resin including an organosiloxane bond and the modified products thereof, a fluorine resin, polyester, polycarbonate, a phenolic resin, and an epoxy resin. The coat resin and the matrix resin may optionally include additives, such as conductive particles. Examples of the conductive particles include particles of metals, such as gold, silver, and copper; and particles of carbon black, titanium oxide, zinc oxide, tin oxide, barium sulfate, aluminum borate, and potassium titanate.

The surfaces of the cores can be coated with a resin by, for example, using a coating-layer forming solution prepared by dissolving the coat resin and, as needed, various types of additives in a suitable solvent. The type of the solvent is not

## 16

limited and may be selected with consideration of the type of the resin used, ease of applying the coating-layer forming solution, and the like.

Specific examples of a method for coating the surfaces of the cores with the coat resin include an immersion method in which the cores are immersed in the coating-layer forming solution; a spray method in which the coating-layer forming solution is sprayed onto the surfaces of the cores; a fluidized-bed method in which the coating-layer forming solution is sprayed onto the surfaces of the cores while the cores are floated using flowing air; and a kneader-coater method in which the cores of the carrier are mixed with the coating-layer forming solution in a kneader coater and subsequently the solvent is removed.

The mixing ratio (i.e., mass ratio) of the toner to the carrier in the two-component developer is preferably toner: carrier=1:100 to 30:100 and is more preferably 3:100 to 20:100.

## 20 Image Forming Apparatus and Image Forming Method

The image forming apparatus according to the exemplary embodiment includes an image holding member; a charging unit that charges the surface of the image holding member; an electrostatic-image formation unit that forms an electrostatic image on the charged surface of the image holding member; a developing unit that includes an electrostatic-image developer and develops the electrostatic image formed on the surface of the image holding member with the electrostatic-image developer to form a toner image; a transfer unit that transfers the toner image formed on the surface of the image holding member onto the surface of a recording medium; a fixing unit that fixes the toner image onto the surface of the recording medium; and a cleaning unit that includes a blade arranged to come into contact with the surface of the image holding member and removes a toner that remains on the surface of the image holding member after transfer of the toner image with the blade.

The image forming apparatus according to the exemplary embodiment uses an image forming method (image forming method according to the exemplary embodiment) including charging the surface of the image holding member; forming an electrostatic image on the charged surface of the image holding member; developing the electrostatic image formed on the surface of the image holding member with the electrostatic-image developer according to the exemplary embodiment to form a toner image; transferring the toner image formed on the surface of the image holding member onto the surface of a recording medium; fixing the toner image onto the surface of the recording medium; and bringing a blade into contact with the surface of the image holding member after transfer of the toner image to remove a toner that remains on the surface of the image holding member.

The image forming apparatus according to the exemplary embodiment may be any image forming apparatus known in the related art, such as a direct-transfer image forming apparatus in which a toner image formed on the surface of an image holding member is directly transferred to a recording medium; an intermediate-transfer image forming apparatus in which a toner image formed on the surface of an image holding member is transferred onto the surface of an intermediate transfer body in the first transfer step and the toner image transferred on the surface of the intermediate transfer body is transferred onto the surface of a recording medium in the second transfer step; and an image forming apparatus including a static-eliminating unit that eliminates static by irradiating the surface of an image holding member

with static-eliminating light subsequent to the transfer of the toner image before the image holding member is again charged.

In the case where the image forming apparatus according to the exemplary embodiment is the intermediate-transfer image forming apparatus, the transfer unit may be constituted by, for example, an intermediate transfer body to which a toner image is transferred, a first transfer subunit that transfers a toner image formed on the surface of the image holding member onto the surface of the intermediate transfer body in the first transfer step, and a second transfer subunit that transfers the toner image transferred on the surface of the intermediate transfer body onto the surface of a recording medium in the second transfer step.

In the image forming apparatus according to the exemplary embodiment, for example, a portion including the developing unit may have a cartridge structure (i.e., process cartridge) detachably attachable to the image forming apparatus. An example of the process cartridge is a process cartridge including the electrostatic-image developer according to the exemplary embodiment and the developing unit.

An example of the image forming apparatus according to the exemplary embodiment is described below, but the image forming apparatus is not limited thereto. Hereinafter, only components illustrated in drawings are described; others are omitted.

FIG. 1 schematically illustrates the image forming apparatus according to the exemplary embodiment.

The image forming apparatus illustrated in FIG. 1 includes first to fourth electrophotographic image formation units **10Y**, **10M**, **10C**, and **10K** that form yellow (Y), magenta (M), cyan (C), and black (K) images, respectively, on the basis of color separation image data. The image formation units (hereinafter, referred to simply as "units") **10Y**, **10M**, **10C**, and **10K** are horizontally arranged in parallel at a predetermined distance from one another. The units **10Y**, **10M**, **10C**, and **10K** may be process cartridges detachably attachable to the image forming apparatus.

An intermediate transfer belt (example of the intermediate transfer body) **20** runs above and extends over the units **10Y**, **10M**, **10C**, and **10K**. The intermediate transfer belt **20** is wound around a drive roller **22** and a support roller **24** and runs clockwise in FIG. 1, that is, in the direction from the first unit **10Y** to the fourth unit **10K**. Using a spring or the like (not illustrated), a force is applied to the support roller **24** in a direction away from the drive roller **22**, thereby applying tension to the intermediate transfer belt **20** wound around the drive roller **22** and the support roller **24**. An intermediate transfer body-cleaning device **30** is disposed so as to come into contact with the image-carrier-side surface of the intermediate transfer belt **20** and to face the drive roller **22**.

Developing devices (examples of the developing units) **4Y**, **4M**, **4C**, and **4K** of the units **10Y**, **10M**, **10C**, and **10K** are supplied with yellow, magenta, cyan, and black toners stored in toner cartridges **8Y**, **8M**, **8C**, and **8K**, respectively.

Since the first to fourth units **10Y**, **10M**, **10C**, and **10K** have the same structure and the same action, the following description is made with reference to, as a representative, the first unit **10Y** that forms an yellow image and is located upstream in a direction in which the intermediate transfer belt runs.

The first unit **10Y** includes a photosensitive member **1Y** serving as an image holding member. The following components are disposed around the photosensitive member **1Y** sequentially in the counterclockwise direction: a charging

roller (example of the charging unit) **2Y** that charges the surface of the photosensitive member **1Y** at a predetermined potential; an exposure device (example of the electrostatic-image formation unit) **3** that forms an electrostatic image by irradiating the charged surface of the photosensitive member **1Y** with a laser beam **3Y** based on a color separated image signal; a developing device (example of the developing unit) **4Y** that develops the electrostatic image by supplying a charged toner to the electrostatic image; a first transfer roller (example of the first transfer subunit) **5Y** that transfers the developed toner image to the intermediate transfer belt **20**; and a photosensitive-member cleaning device (example of the cleaning unit) **6Y** that removes a toner remaining on the surface of the photosensitive member **1Y** after the first transfer.

The photosensitive member cleaning device **6Y** includes a cleaning blade arranged to come into contact with the surface of the photosensitive member **1Y**. The cleaning blade is brought into contact with the surface of the photosensitive member **1Y** that keeps rotating after the transfer of the toner image and removes the toner particles remaining on the surface of the photosensitive member **1Y**.

The first transfer roller **5Y** is disposed so as to be in contact with the inner surface of the intermediate transfer belt **20** and to face the photosensitive member **1Y**. Each of the first transfer rollers **5Y**, **5M**, **5C**, and **5K** of the respective units is connected to a bias power supply (not illustrated) that applies a first transfer bias to the first transfer rollers. Each bias power supply varies the transfer bias applied to the corresponding first transfer roller on the basis of the control by a controller (not illustrated).

The action of forming a yellow image in the first unit **10Y** is described below.

Before the action starts, the surface of the photosensitive member **1Y** is charged at a potential of -600 to -800 V by the charging roller **2Y**.

The photosensitive member **1Y** is formed by stacking a photosensitive layer on a conductive substrate (e.g., volume resistivity at 20° C.:  $1 \times 10^{-6}$  Ωcm or less). The photosensitive layer is normally of high resistance (comparable with the resistance of ordinary resins), but, upon being irradiated with the laser beam, the specific resistance of the portion irradiated with the laser beam varies. Thus, the exposure device **3** irradiates the surface of the charged photosensitive member **1Y** with the laser beam **3Y** on the basis of the image data of the yellow image sent from the controller (not illustrated). As a result, an electrostatic image of yellow image pattern is formed on the surface of the photosensitive member **1Y**.

The term "electrostatic image" used herein refers to an image formed on the surface of the photosensitive member **1Y** by charging, the image being a "negative latent image" formed by irradiating a portion of the photosensitive layer with the laser beam **3Y** to reduce the specific resistance of the irradiated portion such that the charges on the irradiated surface of the photosensitive member **1Y** discharge while the charges on the portion that is not irradiated with the laser beam **3Y** remain.

The electrostatic image, which is formed on the photosensitive member **1Y** as described above, is sent to the predetermined developing position by the rotating photosensitive member **1Y**. The electrostatic image on the photosensitive member **1Y** is developed and visualized in the form of a toner image by the developing device **4Y** at the developing position.

The developing device **4Y** includes an electrostatic-image developer including, for example, at least, a yellow toner

and a carrier. The yellow toner is stirred in the developing device **4Y** to be charged by friction and supported on a developer roller (example of the developer support), carrying an electric charge of the same polarity (i.e., negative) as the electric charge generated on the photosensitive member **1Y**. The yellow toner is electrostatically adhered to the eliminated latent image portion on the surface of the photosensitive member **1Y** as the surface of the photosensitive member **1Y** passes through the developing device **4Y**. Thus, the latent image is developed using the yellow toner. The photosensitive member **1Y** on which the yellow toner image is formed keeps rotating at the predetermined rate, thereby transporting the toner image developed on the photosensitive member **1Y** to the predetermined first transfer position.

Upon the yellow toner image on the photosensitive member **1Y** reaching the first transfer position, first transfer bias is applied to the first transfer roller **5Y** so as to generate an electrostatic force on the toner image in the direction from the photosensitive member **1Y** toward the first transfer roller **5Y**. Thus, the toner image on the photosensitive member **1Y** is transferred to the intermediate transfer belt **20**. The transfer bias applied has the opposite polarity (+) to that of the toner (-) and controlled to be, in the first unit **10Y**, for example, +10  $\mu$ A by a controller (not illustrated).

After the transfer of the toner image, the photosensitive member **1Y** keeps rotating and is brought into contact with the cleaning blade included in the photosensitive member cleaning device **6Y**. The toner particles remaining on the photosensitive member **1Y** are removed by the photosensitive-member cleaning device **6Y** and then collected.

Each of the first transfer biases applied to first transfer rollers **5M**, **5C**, and **5K** of the second, third, and fourth units **10M**, **10C**, and **10K** is controlled in accordance with the first unit **10Y**.

Thus, the intermediate transfer belt **20**, on which the yellow toner image is transferred in the first unit **10Y**, is successively transported through the second to fourth units **10M**, **10C**, and **10K** while toner images of the respective colors are stacked on top of another.

The resulting intermediate transfer belt **20** on which toner images of four colors are multiple-transferred in the first to fourth units is then transported to a second transfer section including a support roller **24** being in contact with the inner surface of the intermediate transfer belt **20** and a second transfer roller (example of the second transfer subunit) **26** disposed on the image-carrier-side of the intermediate transfer belt **20**. A recording paper (example of the recording medium) **P** is fed by a feed mechanism into a narrow space between the second transfer roller **26** and the intermediate transfer belt **20** that are brought into contact with each other at the predetermined timing. The second transfer bias is then applied to the support roller **24**. The transfer bias applied here has the same polarity (-) as that of the toner (-) and generates an electrostatic force on the toner image in the direction from the intermediate transfer belt **20** toward the recording paper **P**. Thus, the toner image on the intermediate transfer belt **20** is transferred to the recording paper **P**. The intensity of the second transfer bias applied is determined on the basis of the resistance of the second transfer section which is detected by a resistance detector (not illustrated) that detects the resistance of the second transfer section and controlled by changing voltage.

Subsequently, the recording paper **P** is transported into a nip part of the fixing device (example of the fixing unit) **28** at which a pair of fixing rollers are brought into contact with each other. The toner image is fixed to the recording paper **P** to form a fixed image.

Examples of the recording paper **P** to which a toner image is transferred include plain paper used in electrophotographic copiers, printers, and the like. Instead of the recording paper **P**, OHP films and the like may be used as a recording medium.

The surface of the recording paper **P** may be smooth in order to enhance the smoothness of the surface of the fixed image. Examples of such a recording paper include coated paper produced by coating the surface of plain paper with resin or the like and art paper for printing.

The recording paper **P**, to which the color image has been fixed, is transported toward an exit portion. Thus, the series of the steps for forming a color image are terminated.

#### Process Cartridge and Toner Cartridge

The process cartridge according to the exemplary embodiment includes an image holding member, a developing unit that includes the electrostatic-image developer according to the exemplary embodiment and develops an electrostatic image formed on the surface of an image holding member with the electrostatic-image developer to form a toner image, and a cleaning unit that includes a blade arranged to come into contact with the surface of the image holding member and removes a toner that remains on the surface of the image holding member after transfer of the toner image with the blade. The process cartridge according to the exemplary embodiment is detachably attachable to an image forming apparatus.

The structure of the process cartridge according to the exemplary embodiment is not limited to the above-described one. The process cartridge according to the exemplary embodiment may further include at least one unit selected from a charging unit, an electrostatic-image formation unit, a transfer unit, and the like.

An example of the process cartridge according to the exemplary embodiment is described below, but the process cartridge is not limited thereto. Hereinafter, only components illustrated in FIG. 2 are described; others are omitted.

FIG. 2 schematically illustrates the process cartridge according to the exemplary embodiment.

A process cartridge **200** illustrated in FIG. 2 includes, for example, a photosensitive member **107** (example of the image holding member), a charging roller **108** (example of the charging unit) disposed on the periphery of the photosensitive member **107**, a developing device **111** (example of the developing unit), and a photosensitive-member cleaning device **113** (example of the cleaning unit), which are combined into one unit using a housing **117** to form a cartridge. The housing **117** has an aperture **118** for exposure. A mounting rail **116** is disposed on the housing **117**. The photosensitive-member cleaning device **113** includes a blade arranged to come into contact with the photosensitive member **107**.

In FIG. 2, Reference numeral **109** denotes an exposure device (example of the electrostatic-image formation unit), Reference numeral **112** denotes a transfer device (example of the transfer unit), Reference numeral **115** denotes a fixing device (example of the fixing unit), and the Reference numeral **300** denotes recording paper (example of the recording medium).

The toner cartridge according to an exemplary embodiment is described below.

The toner cartridge according to the exemplary embodiment includes the toner according to the exemplary embodiment and is detachably attachable to an image forming apparatus. The toner cartridge includes a replacement toner that is to be supplied to the developing unit disposed inside an image forming apparatus.

The image forming apparatus illustrated in FIG. 1 is an image forming apparatus that includes the toner cartridges **8Y**, **8M**, **8C**, and **8K** detachably attached to the image forming apparatus. Each of the developing devices **4Y**, **4M**, **4C**, and **4K** is connected to a specific one of the toner cartridges which corresponds to the developing device (color) with a toner feed pipe (not illustrated). When the amount of toner contained in a toner cartridge is small, the toner cartridge is replaced.

## EXAMPLES

Details of the exemplary embodiment of the present disclosure are described below with reference to Examples below. The exemplary embodiment of the present disclosure is not limited to Examples below. Hereinafter, the terms "part" and "%" are on a mass basis unless otherwise specified.

## Preparation of Toner Particles

## Preparation of Amorphous Polyester Resin Dispersion Liquid (A1)

Terephthalic acid: 70 parts

Fumaric acid: 30 parts

Ethylene glycol: 44 parts

1,5-Pentanediol: 46 parts

Into a flask equipped with a stirring device, a nitrogen introducing tube, a temperature sensor, and a fractionating column, the above materials are charged. Under a nitrogen stream, the temperature is increased to 210° C. over 1 hour, and 1 part of titanium tetraethoxide relative to 100 parts of the total amount of the above materials is added to the flask. While the product water is removed by distillation, the temperature is increased to 240° C. over 0.5 hours and dehydration condensation is continued for 1 hour at 240° C. Subsequently, the product of the reaction is cooled. Hereby, an amorphous polyester resin having a weight-average molecular weight of 94,500 and a glass transition temperature of 61° C. is prepared.

Into a container equipped with a temperature control unit and a nitrogen purging unit, 40 parts of ethyl acetate and 25 parts of 2-butanol are charged to form a mixed solvent. To the mixed solvent, 100 parts of the amorphous polyester resin is gradually added and dissolved in the mixed solvent. To the resulting solution, a 10% aqueous ammonia solution is added in an amount 3 times by mole with respect to the acid value of the resin. The resulting mixture is stirred for 30 minutes. Then, the inside of the container is purged with dry nitrogen. While the temperature is maintained to be 40° C. and the liquid mixture is stirred, 400 parts of ion-exchange water is added dropwise to the container in order to perform emulsification. After the addition of ion-exchange water has been terminated, the resulting emulsion is cooled to 25° C. Hereby, a resin particle dispersion liquid that includes resin particles having a volume-average particle size of 210 nm dispersed therein is prepared. Ion-exchange water is added to the resin particle dispersion liquid to adjust the solid content in the dispersion liquid to be 20%. Hereby, an amorphous polyester resin dispersion liquid (A1) is prepared.

## Preparation of Crystalline Polyester Resin Dispersion Liquid (B1)

Dimethyl sebacate: 97 parts

Sodium dimethyl-5-sulfonate isophthalate: 3 parts

Ethylene glycol: 100 parts

Dibutyltin oxide (catalyst): 0.3 parts

The above materials are charged into a three-necked flask dried by heating. Subsequently, the atmosphere inside the

three-necked flask is replaced with an inert atmosphere by purging with a nitrogen gas. The resulting mixture is stirred by mechanical stirring and caused to reflux at 180° C. for 5 hours. Then, the temperature is gradually increased to 240° C. under reduced pressure and stirring is performed for 2 hours. When the mixture becomes viscous, air cooling is performed and the reaction is stopped. Hereby, a crystalline polyester resin having a weight-average molecular weight of 9,700 and a melting temperature of 84° C. is prepared.

10 Then, 90 parts of the crystalline polyester resin, 1.8 parts of an anionic surfactant "Neogen RK" produced by DKS Co. Ltd., and 210 parts of ion-exchange water are mixed with one another. The resulting mixture is heated to 100° C. and dispersed with a homogenizer "ULTRA-TURRAX T50" produced by IKA. Subsequently, a dispersion treatment is performed for 1 hour using a pressure-discharge Gaulin homogenizer. Hereby, a resin particle dispersion liquid that includes resin particles having a volume-average particle size of 205 nm dispersed therein is prepared. Ion-exchange water is added to the resin particle dispersion liquid in order to adjust the solid content in the dispersion liquid to be 20%. Hereby, a crystalline polyester resin dispersion liquid (B1) is prepared.

## Preparation of Release Agent Particle Dispersion Liquid (W1)

Paraffin wax "HNP-9" produced by Nippon Seiro Co., Ltd.: 100 parts

Anionic surfactant "Neogen RK" produced by Dai-ichi Kogyo Seiyaku Co., Ltd.: 1 part

30 Ion-exchange water: 350 parts

The above materials are mixed with one another and heated to 100° C. The resulting mixture is dispersed with a homogenizer "ULTRA-TURRAX T50" produced by IKA and then further dispersed with a pressure-discharge Gaulin homogenizer. Hereby, a release agent particle dispersion liquid in which release agent particles having a volume-average particle size of 200 nm are dispersed is prepared. Ion-exchange water is added to the release agent particle dispersion liquid in order to adjust the solid content in the dispersion liquid to be 20%. Hereby, a release agent particle dispersion liquid (W1) is prepared.

## Preparation of Colorant Particle Dispersion Liquid (K1)

Carbon black "Regal330" produced by Cabot Corporation: 50 parts

45 Ionic surfactant "Neogen RK" produced by DKS Co. Ltd.: 5 parts

Ion-exchange water: 195 parts

The above materials are mixed with one another, and the resulting mixture is dispersed with Ultimizer produced by Sugino Machine Limited at 240 MPa for 10 minutes. Hereby, a colorant particle dispersion liquid (K1) having a solid content of 20% is prepared.

## Preparation of Toner Particles

Ion-exchange water: 200 parts

55 Amorphous polyester resin dispersion liquid (A1): 150 parts

Crystalline polyester resin dispersion liquid (B1): 10 parts

Release agent particle dispersion liquid (W1): 10 parts

Colorant particle dispersion liquid (K1): 15 parts

60 Anionic surfactant (TaycaPower): 2.8 parts

The above materials are charged into a round-bottom flask made of stainless steel. After the pH has been adjusted to be 3.5 by addition of 0.1 N nitric acid, an aqueous polyaluminum chloride solution prepared by dissolving 2 parts of polyaluminum chloride (30% powder produced by Oji Paper Co., Ltd.) in 30 parts of ion-exchange water is added to the flask. After dispersion has been performed with a homog-

enizer “ULTRA-TURRAX T50” produced by IKA at 30° C., the temperature is increased to 45° C. in a heating oil bath. Then, holding is performed until the volume-average particle size reaches 4.9  $\mu\text{m}$ . Subsequently, 60 parts of the amorphous polyester resin dispersion liquid (A1) is added to the flask and holding is performed for 30 minutes. When the volume-average particle size reaches 5.2  $\mu\text{m}$ , another 60 parts of the amorphous polyester resin dispersion liquid (A1) is added to the flask and holding is performed for 30 minutes. Then, 20 parts of a 10% aqueous solution of nitrilotriacetic acid (NTA) metal salt “Chelest 70” produced by Chelest Corporation is added to the flask. Subsequently, the pH is adjusted to be 9.0 by addition of a 1 N aqueous sodium hydroxide solution. Then, 1 part of an anionic surfactant “TaycaPower” is added to the flask. While stirring is continued, the temperature is increased to 85° C. and then holding is performed for 5 hours. Subsequently, the temperature is reduced to 20° C. at a rate of 20° C./min. Then, filtration is performed. The resulting substance is sufficiently washed with ion-exchange water and dried to form toner particles (1) having a volume-average particle size of 5.7  $\mu\text{m}$  and an average circularity of 0.971.

#### Preparation of Layered Compound Particles

##### Preparation of Melamine Cyanurate Particles

Commercial melamine cyanurate particles are disintegrated and classified with a jet mill to prepare the melamine cyanurate particles (1) to (11) described below. In Table 1, “MC” means melamine cyanurate.

Melamine cyanurate particles (1): number-average particle size: 0.70  $\mu\text{m}$

Melamine cyanurate particles (2): number-average particle size: 0.32  $\mu\text{m}$

Melamine cyanurate particles (3): number-average particle size: 0.35  $\mu\text{m}$

Melamine cyanurate particles (4): number-average particle size: 0.40  $\mu\text{m}$

Melamine cyanurate particles (5): number-average particle size: 1.50  $\mu\text{m}$

Melamine cyanurate particles (6): number-average particle size: 1.80  $\mu\text{m}$

Melamine cyanurate particles (7): number-average particle size: 2.10  $\mu\text{m}$

Melamine cyanurate particles (8): number-average particle size: 2.50  $\mu\text{m}$

Melamine cyanurate particles (9): number-average particle size: 2.80  $\mu\text{m}$

Melamine cyanurate particles (10): number-average particle size: 3.00  $\mu\text{m}$

Melamine cyanurate particles (11): number-average particle size: 3.50  $\mu\text{m}$

##### Preparation of Boron Nitride Particles

Commercial boron nitride particles are disintegrated and classified with a jet mill to prepare the boron nitride particles having a number-average particle size of 0.70  $\mu\text{m}$ . In Table 1, “BN” means boron nitride.

##### Preparation of Molybdenum Disulfide Particles

Commercial molybdenum disulfide particles are disintegrated and classified with a jet mill to prepare the molybdenum disulfide particles having a number-average particle size of 0.70  $\mu\text{m}$ . In Table 1, “MoS<sub>2</sub>” means molybdenum disulfide.

##### Preparation of Silica Particles

Silica particles are prepared by the sol-gel method. The silica particles are rendered hydrophobic with hexamethyl-disilazane and classified as needed. Hereby, the following silica particles are prepared.

Silica particles (1): number-average particle size: 0.09  $\mu\text{m}$ , average circularity: 0.950

Silica particles (2): number-average particle size: 0.09  $\mu\text{m}$ , average circularity: 0.920

Silica particles (3): number-average particle size: 0.09  $\mu\text{m}$ , average circularity: 0.980

Silica particles (4): number-average particle size: 0.06  $\mu\text{m}$ , average circularity: 0.950

Silica particles (5): number-average particle size: 0.29  $\mu\text{m}$ , average circularity: 0.950

Silica particles (6): number-average particle size: 0.09  $\mu\text{m}$ , average circularity: 0.890

Silica particles (7): number-average particle size: 0.30  $\mu\text{m}$ , average circularity: 0.950

Silica particles (8): number-average particle size: 0.20  $\mu\text{m}$ , average circularity: 0.950

Silica particles (9): number-average particle size: 0.07  $\mu\text{m}$ , average circularity: 0.950

Silica particles (10): number-average particle size: 0.19  $\mu\text{m}$ , average circularity: 0.950

Silica particles (11): number-average particle size: 0.45  $\mu\text{m}$ , average circularity: 0.950

Silica particles (12): number-average particle size: 0.23  $\mu\text{m}$ , average circularity: 0.950

Silica particles (13): number-average particle size: 0.27  $\mu\text{m}$ , average circularity: 0.950

##### Preparation of Carriers

After 500 parts of spherical magnetite powder particles (volume-average particle size: 0.55  $\mu\text{m}$ ) have been stirred with a Henschel mixer, 5 parts of a titanate coupling agent is added. The resulting mixture is heated to 100° C. and then stirred for 30 minutes. Subsequently, 6.25 parts of phenol, 9.25 parts of 35% formalin, 500 parts of magnetite particles treated with a titanate coupling agent, 6.25 parts of 25% ammonia water, and 425 parts of water are charged into a four-necked flask. While the resulting mixture is stirred, the reaction is conducted at 85° C. for 120 minutes. Then, the temperature is reduced to 25° C. After 500 parts of water has been added to the flask, the resulting supernatant is removed and the precipitate is washed with water. The precipitate is dried by heating under reduced pressure to form a carrier having an average particle size of 35  $\mu\text{m}$ .

#### Example 1

The toner particles (1), the melamine cyanurate particles (1), and the silica particles (1) are charged into a sample mill at the proportions described in Table 1. The resulting mixture is stirred at 10,000 rpm for 30 seconds. Subsequently, screening is performed with a vibration sieve having an opening of 45  $\mu\text{m}$ . Hereby, a toner having a volume-average particle size of 5.7  $\mu\text{m}$  is prepared.

The toner and the carrier are charged into a V-blender at a mass ratio of Toner:Carrier=5:95. The resulting mixture is stirred for 20 minutes to form a developer.

#### Examples 2 to 19 and Comparative Examples 1 to 3

Toners and developers are prepared as in Example 1, except that the type and amount of the layered compound particles used and the type and amount of the silica particles used are changed.

##### Performance Evaluations

Colored Streaks in High-Temperature, High-Humidity Environment

An image having an area coverage of 40% is formed on 100,000 A4 size paper sheets with a modification of “700 Digital Color Press” produced by Fuji Xerox Co., Ltd. at 28° C. and a relative humidity of 85%. Subsequently, a full halftone image chart is formed on 500 A4 size paper sheets. The 10th, 50th, 100th, and 500th paper sheets are visually

inspected and the total number of colored streaks formed in the halftone images is counted and classified in the following manner.

G1: No colored streaks

G2: 1 colored streak

G3: 2 to 5 colored streaks, acceptable

G4: 6 or more colored streaks, not acceptable in the practical use

#### Aggregates in Cleaning Box

After the formation of the images described above, the contents of a cleaning box of the photosensitive member are taken and screened through a sieve having an opening of 45  $\mu\text{m}$ . The number of the aggregates is counted.

G1: No aggregate

G2: 1 to 5 aggregates

G3: 6 to 19 aggregates

G4: 20 or more aggregates

wherein the inorganic particles have an average circularity of 0.910 or more and 0.995 or less, and

wherein a ratio Da/Db of a number-average particle size Da of the layered compound particles to a number-average particle size Db of the inorganic particles is 1.2 or more and 43 or less.

5 2. The electrostatic-image developing toner according to claim 1,

10 wherein the ratio Da/Db of the number-average particle size Da of the layered compound particles to the number-average particle size Db of the inorganic particles is 5 or more and 43 or less.

15 3. The electrostatic-image developing toner according to claim 2,

wherein a mass ratio Mb/Ma of a content Mb of the inorganic particles to a content Ma of the layered compound particles is 0.1 or more and 500 or less.

TABLE 1

| Layered compound particles |                  |                              |                         | Inorganic particles |          |                              |                     |                         |                 |            |                         |    |
|----------------------------|------------------|------------------------------|-------------------------|---------------------|----------|------------------------------|---------------------|-------------------------|-----------------|------------|-------------------------|----|
| Type                       | Compound         | Number-average particle size | Content in entire toner | Type                | Compound | Number-average particle size | Average circularity | Content in entire toner | Particle size   | Amount     | Performance evaluations |    |
|                            |                  | Da ( $\mu\text{m}$ )         | Ma (mass %)             |                     |          | Db ( $\mu\text{m}$ )         | ratio Da/Db         | ratio Mb/Ma             | Colored streaks | Aggregates |                         |    |
| Comparative example 1      | (10) MC          | 3.00                         | 0.2                     | (4)                 | Silica   | 0.06                         | 0.950               | 2.0                     | 50.0            | 10         | G4                      | G4 |
| Comparative example 2      | (2) MC           | 0.32                         | 0.2                     | (5)                 | Silica   | 0.29                         | 0.950               | 2.0                     | 1.1             | 10         | G4                      | G4 |
| Comparative example 3      | (1) MC           | 0.70                         | 0.2                     | (6)                 | Silica   | 0.09                         | 0.890               | 2.0                     | 7.8             | 10         | G4                      | G4 |
| Example 1                  | (1) MC           | 0.70                         | 0.2                     | (1)                 | Silica   | 0.09                         | 0.950               | 2.0                     | 7.8             | 10         | G2                      | G2 |
| Example 2                  | (1) MC           | 0.70                         | 0.2                     | (2)                 | Silica   | 0.09                         | 0.920               | 2.0                     | 7.8             | 10         | G2                      | G2 |
| Example 3                  | (1) MC           | 0.70                         | 0.2                     | (3)                 | Silica   | 0.09                         | 0.980               | 2.0                     | 7.8             | 10         | G1                      | G1 |
| Example 4                  | (3) MC           | 0.35                         | 0.2                     | (7)                 | Silica   | 0.30                         | 0.950               | 2.0                     | 1.2             | 10         | G3                      | G3 |
| Example 5                  | (3) MC           | 0.35                         | 0.2                     | (8)                 | Silica   | 0.20                         | 0.950               | 2.0                     | 1.8             | 10         | G3                      | G3 |
| Example 6                  | (4) MC           | 0.40                         | 0.2                     | (8)                 | Silica   | 0.20                         | 0.950               | 2.0                     | 2.0             | 10         | G3                      | G3 |
| Example 7                  | (8) MC           | 2.50                         | 0.2                     | (9)                 | Silica   | 0.07                         | 0.950               | 2.0                     | 35.7            | 10         | G1                      | G1 |
| Example 8                  | (9) MC           | 2.80                         | 0.2                     | (9)                 | Silica   | 0.07                         | 0.950               | 2.0                     | 40.0            | 10         | G1                      | G1 |
| Example 9                  | (10) MC          | 3.00                         | 0.2                     | (9)                 | Silica   | 0.07                         | 0.950               | 2.0                     | 42.9            | 10         | G1                      | G1 |
| Example 10                 | (5) MC           | 1.50                         | 0.2                     | (10)                | Silica   | 0.19                         | 0.950               | 2.0                     | 7.8             | 10         | G3                      | G3 |
| Example 11                 | (11) MC          | 3.50                         | 0.2                     | (11)                | Silica   | 0.45                         | 0.950               | 2.0                     | 7.8             | 10         | G2                      | G2 |
| Example 12                 | (6) MC           | 1.80                         | 0.2                     | (12)                | Silica   | 0.23                         | 0.950               | 2.0                     | 7.8             | 10         | G3                      | G3 |
| Example 13                 | (7) MC           | 2.10                         | 0.2                     | (13)                | Silica   | 0.27                         | 0.950               | 2.0                     | 7.8             | 10         | G2                      | G2 |
| Example 14                 | (1) MC           | 0.70                         | 1.5                     | (1)                 | Silica   | 0.09                         | 0.950               | 2.0                     | 7.8             | 1.3        | G2                      | G2 |
| Example 15                 | (1) MC           | 0.70                         | 3.0                     | (1)                 | Silica   | 0.09                         | 0.950               | 2.0                     | 7.8             | 0.7        | G3                      | G3 |
| Example 16                 | (1) MC           | 0.70                         | 0.01                    | (1)                 | Silica   | 0.09                         | 0.950               | 5.0                     | 7.8             | 500        | G1                      | G1 |
| Example 17                 | (1) MC           | 0.70                         | 3.0                     | (1)                 | Silica   | 0.09                         | 0.950               | 0.3                     | 7.8             | 0.1        | G3                      | G3 |
| Example 18                 | BN               | 0.70                         | 0.2                     | (1)                 | Silica   | 0.09                         | 0.950               | 2.0                     | 7.8             | 10         | G1                      | G1 |
| Example 19                 | MoS <sub>2</sub> | 0.70                         | 0.2                     | (1)                 | Silica   | 0.09                         | 0.950               | 2.0                     | 7.8             | 10         | G2                      | G2 |

The foregoing description of the exemplary embodiment of the present disclosure has been provided for the purposes of illustration and description. It is not intended to be exhaustive or to limit the disclosure to the precise forms disclosed. Obviously, many modifications and variations will be apparent to practitioners skilled in the art. The embodiment was chosen and described in order to best explain the principles of the disclosure and its practical applications, thereby enabling others skilled in the art to understand the disclosure for various embodiments and with the various modifications as are suited to the particular use contemplated. It is intended that the scope of the disclosure be defined by the following claims and their equivalents.

What is claimed is:

1. An electrostatic-image developing toner comprising: toner particles; layered compound particles; and inorganic particles,

50 4. The electrostatic-image developing toner according to claim 3,

wherein the mass ratio Mb/Ma of the content Mb of the inorganic particles to the content Ma of the layered compound particles is 1 or more and 500 or less.

55 5. The electrostatic-image developing toner according to claim 2,

wherein the inorganic particles include silica particles.

60 6. The electrostatic-image developing toner according to claim 1,

wherein a mass ratio Mb/Ma of a content Mb of the inorganic particles to a content Ma of the layered compound particles is 0.1 or more and 500 or less.

65 7. The electrostatic-image developing toner according to claim 6,

wherein the mass ratio Mb/Ma of the content Mb of the inorganic particles to the content Ma of the layered compound particles is 1 or more and 500 or less.

27

8. The electrostatic-image developing toner according to claim 1,  
 wherein a content of the layered compound particles is 0.01% by mass or more and 5.0% by mass or less of a total amount of the electrostatic-image developing toner. 5
9. The electrostatic-image developing toner according to claim 8,  
 wherein the content of the layered compound particles is 0.01% by mass or more and 0.5% by mass or less of the total amount of the electrostatic-image developing toner. 10
10. The electrostatic-image developing toner according to claim 1,  
 wherein the number-average particle size Da of the layered compound particles is 0.3  $\mu\text{m}$  or more and 5.0  $\mu\text{m}$  or less. 15
11. The electrostatic-image developing toner according to claim 10,  
 wherein the number-average particle size Da of the layered compound particles is 0.4  $\mu\text{m}$  or more and 2.0  $\mu\text{m}$  or less. 20
12. The electrostatic-image developing toner according to claim 1,  
 wherein the number-average particle size Db of the inorganic particles is 0.06  $\mu\text{m}$  or more and 0.3  $\mu\text{m}$  or less. 25
13. The electrostatic-image developing toner according to claim 12,  
 wherein the number-average particle size Db of the inorganic particles is 0.07  $\mu\text{m}$  or more and 0.2  $\mu\text{m}$  or less. 30
14. The electrostatic-image developing toner according to claim 1,  
 wherein the layered compound particles include at least one type of particles selected from the group consisting of melamine cyanurate particles, boron nitride particles, graphite fluoride particles, molybdenum disulfide particles, and mica particles. 35
15. The electrostatic-image developing toner according to claim 1,  
 wherein the inorganic particles include silica particles. 40
16. An electrostatic-image developer comprising the electrostatic-image developing toner according to claim 1. 45
17. A process cartridge detachably attachable to an image forming apparatus, the process cartridge comprising:  
 an image holding member;  
 a developing unit that includes the electrostatic-image developer according to claim 16 and develops an electrostatic image formed on a surface of the image holding member with the electrostatic-image developer to form a toner image; and

28

- a cleaning unit that includes a blade arranged to come into contact with the surface of the image holding member and removes a toner that remains on the surface of the image holding member after transfer of the toner image with the blade.
18. An image forming apparatus comprising:  
 an image holding member;  
 a charging unit that charges a surface of the image holding member;  
 an electrostatic-image formation unit that forms an electrostatic image on the charged surface of the image holding member;  
 a developing unit that includes the electrostatic-image developer according to claim 16 and develops the electrostatic image formed on the surface of the image holding member with the electrostatic-image developer to form a toner image;  
 a transfer unit that transfers the toner image formed on the surface of the image holding member onto a surface of a recording medium;  
 a fixing unit that fixes the toner image transferred on the surface of the recording medium; and  
 a cleaning unit that includes a blade arranged to come into contact with the surface of the image holding member and removes a toner that remains on the surface of the image holding member after transfer of the toner image with the blade.
19. An image forming method comprising:  
 charging a surface of an image holding member;  
 forming an electrostatic image on the charged surface of the image holding member;  
 developing the electrostatic image formed on the surface of the image holding member with the electrostatic-image developer according to claim 16 to form a toner image;  
 transferring the toner image formed on the surface of the image holding member onto a surface of a recording medium;  
 fixing the toner image transferred on the surface of the recording medium; and  
 bringing a blade into contact with the surface of the image holding member after transfer of the toner image to remove a toner that remains on the surface of the image holding member.
20. A toner cartridge detachably attachable to an image forming apparatus, the toner cartridge comprising the electrostatic-image developing toner according to claim 1.

\* \* \* \* \*